

## UNITED STATES PATENT OFFICE

MAXIMILIAN PAUL SCHMIDT, RUDOLF ZAHN, AND WILHELM KRIEGER, OF WIES-BADEN-BIEBRICH, GERMANY, ASSIGNORS TO HALLE & CO. AKTIENGESELLSCHAFT, A CORPORATION OF GERMANY

## PROCESS OF PREPARING PICTURES TO BE PRODUCED BY TANNING ACTION

No Drawing. Application filed August 7, 1928, Serial No. 298,126, and in Germany August 22, 1927.

Our present invention relates to the preparation of pictures to be produced by the action of tanning substances.

In certain photo printing processes (for instance pigment-printing, gum printing, ozotypic printing or the like) and also in many other arts of printing (copper-deep printing, photo-lithography, photo-printing, etc.), the layers prepared with salts of chromic acid take a prominent place in spite of the disadvantages they show, the most serious drawback being that, notwithstanding the many attempts made in this respect (see for instance Namias, Eders Jahrbuch, 1904, page 142), it has not been possible to stabilize the colloid layer sensitized with chromates before exposure to light so as to render them suitable for technical purposes.

Colloid layers sensitized by means of salts of chromic acid are not only unfit for being stored for some time, for even in the course of a few hours the said layers may under unfavorable atmospheric conditions undergo so extensive alterations that it is no longer possible to obtain invariably good results by using them for the above mentioned purposes.

Although attempts have been made to substitute for the chromates other bodies (see Strasser German Patent No. 160,729, issued April 10, 1905) the use of such other bodies has not been adopted in practice owing to the unsatisfactory photographic results they gave.

We have now found that the decomposition products of diazo compounds which are formed during exposure to light are capable, when subjected to reaction with chromates or any other substance, in the presence of a colloid, of producing a tanning action. By the term "tanning action" is here to be understood that action by which the solubility or the swelling up of colloids is diminished. A similar action to that of a bichromate can be produced by other oxidation agents for instance ammonium hypobromite, and likewise diazo compounds of great coupling capacity. In using stable diazo compounds as for instance ortho- or para-hydroxy- or amino-diazo compounds it has

been found that layers sensitized therewith are, when not yet exposed to light, of a better stability than layers prepared from chromates. Moreover the new process is applicable to a much greater variety of purposes because sensitized papers prepared according to this process can be kept in store fit for immediate use so that they need not be freshly sensitized whenever they are to be employed. The great number of available diazo compounds enables one, by conveniently varying the process, to modify extensively the gradation of the light-sensitive layers.

The diazo compounds in question may be incorporated into the colloid layer when it is being prepared or by subsequently placing the layer in a bath prepared from a solution of the respective diazo compound, if required, with a stabilizer or sensitizer added thereto. The said diazo compounds may also be applied alone on a suitable base (for instance paper, films, metal-foils or the like), then exposed to light under a corresponding original and finally pressed upon a colloid layer moistened with a solution of a chromate.

Diazo compounds may be used with advantage instead of chromates in all reproducing processes where a tanning effect is to be produced on colloid layer by chromates reduced by the action of the light. Among those processes may be mentioned: Pigment-printing, copper-deep printing, photolithography, phototypy, gelatine-printing, gum-printing. Of course, in the new process, all methods practiced in the utilization of chromate layers for preparing pictures may be used. Thus, the layers in question may contain pigments of every kind. They may, as is usual in the pertaining arts, be colored with color solutions before or after they have been washed. In certain cases it is advantageous to color the layers before and also after washing them. Furthermore there may be rolled on the layers in question, after being exposed to light, a fatty color, or only a varnish, then the layer developed with warm water and, if desired, dusted over with a color dust in order to intensify the picture.

The following examples serve to illustrate our invention, but are not intended to limit it thereto.

1. Pigment paper is placed in a bath prepared with a solution, at 18° C. temperature, of 4 parts of hydrofluoborate of 1-diazo-4-dimethylaminobenzene in 100 parts of water and left therein until it is thoroughly moistened; the paper is then pressed upon a well cleaned glass-plate and dried and, after drying, it is detached from the latter. The said diazo compound may be obtained by diazotizing 1-amino-4-dimethylaminobenzene in the presence of a hydrofluoboric acid. After drying, the dried pigment paper is exposed to light under a negative, then placed together with a suitable piece of transfer paper in a 2 per cent solution of potassium bichromate, until the pigment paper becomes stretched, the pigment paper and transfer paper are then taken from the bath, pressed upon each other and the picture is developed by dissolving therefrom the gelatine which has not been exposed to light in water of about 40° C. temperature in the manner in which pigment-pictures are usually developed.

2. 4 parts of 4-diazo-3-methyl-4-dimethyl-anilinsulfate obtained by diazotizing 4-amino-3-methyl-1-dimethylanilin in a sulfuric solution, are dissolved in 100 parts of water and this solution is spread on well-sized paper having a smooth surface. After drying, the paper so treated is exposed to light under a diapositive decomposed through a dotted screen. The paper after exposure to light is pressed upon pigment paper moistened with a 0.25 per cent solution of potassium bichromate and pressed out, such as it is used for copper etchings (so-called etching paper), the paper is then drawn off after about one minute and pressed immediately upon the copper plate or copper-cylinder intended to receive the etching. On the copper the picture is developed as usual with water of a temperature of 40° C. and then, after drying, etched with ferric chloride.

Instead of 4-diazo-3-methyl-4-dimethyl-anilinsulfate there may be used the cadmium salt of 1-diazo-4-monoethylnaphthylamine or the diazo compound of para-amino-diphenylamine.

3. So-called Albert's autotypy-paper is placed in a bath prepared from a solution of 4 parts of the diazo compound from 1-amino-2-oxy-acetylarnino-5-benzenesulfonic acid in 100 parts of water, dried on a glass plate, then exposed to light under a negative decomposed, through a dotted screen, placed in a bath prepared from a 2% solution of potassium bichromate and finally thoroughly watered. On the picture when dry is applied by a roller a photolithographic re-printing color giving a uni-

formly grey tone and then placed in water. When the paper has become sufficiently moist, the picture can be developed by means of a wet small piece of wadding; after drying the developed picture it is further re-printed by the usual method on a lithographic stone, zinc or aluminium and further treated.

4. A photo-print film, produced from nitrocellulose with a gelatine layer of a suitable degree of hardness, such as the known "Agfa" film, is placed in a bath prepared from 4 parts of the diazo compound from 1-amino-2-oxy-3-naphthalenecarboxylic acid in 100 parts of water and a small quantity of ammonia, then drawn through acetic acid and by drying it at 28—29° C. a wrinkled grain is produced thereon. Upon the film so prepared a negative is copied, the film exposed to light and then placed for 2 minutes in a bath prepared from a 2% solution of potassium bichromate, whereupon it is thoroughly watered and dried. The further treatment and printing are operated in the usual manner.

5. 10 parts of gelatine, 2 parts of colcothar red iron oxide, 2 parts of sugar and 60 parts of water are made up into an emulsion and there is then added a solution, acidified with diluted hydrochloric acid, of 0.5 parts of a diazo compound obtained by diazotizing 1-amino-4-phenylaminobenzene in a hydrochloric solution and 1.5 parts of sodium 1,3,6-naphthalenetrisulfonate in 20 parts of water; the emulsion thus obtained is poured on paper in the usual manner and the latter dried, exposed to light and further treated as indicated in Example 2.

In the following claims by the term "tanning action" is to be understood that action by which the solubility and the swelling up of colloids are diminished under the influence of light.

By the term "tanning agent" are to be understood ammonium hypobromite, etc., and likewise diazo compounds of great coupling capacity.

We claim:

1. The process of preparing pictures to be produced by tanning action consisting in applying a mixture of a diazo compound and an organic colloid on a base placing the object to be copied on the layer sensitive to light, exposing it to light, treating it with a tanning agent and developing it with water.

2. The process of preparing pictures to be produced by tanning action consisting in applying a mixture of a diazo compound, an organic colloid and a pigment on a base placing the object to be copied on the layer sensitive to light, exposing it to light, treating it with a tanning agent and developing it with water.

3. The process of preparing pictures to be produced by tanning action consisting in applying a mixture of a diazo compound, an organic colloid, a pigment and a stabilizer on a base placing the object to be copied on the layer sensitive to light, exposing it to light, treating it with a tanning agent and developing it with water. 70
4. The process of preparing pictures to be produced by tanning action consisting in applying a mixture of a diazo compound and an organic colloid on a base placing the object to be copied on the layer sensitive to light, exposing it to light, treating it with a solution of a chromate and developing it with water. 75
5. The process of preparing pictures to be produced by tanning action consisting in applying a mixture of a diazo compound, an organic colloid and a pigment on a base placing the object to be copied on the layer sensitive to light, exposing it to light, treating it with a solution of a chromate and developing it with water. 80
6. The process of preparing pictures to be produced by tanning action consisting in applying a mixture of a diazo compound, an organic colloid, a pigment and a stabilizer on a base placing the object to be copied on the layer sensitive to light, exposing it to light, treating it with a solution of a chromate and developing it with water. 85
7. The process of preparing pictures to be produced by tanning action consisting in applying a mixture of a diazo compound containing besides the diazo group a basic group and an organic colloid on a base placing the object to be copied on the layer sensitive to light, exposing it to light, treating it with a tanning agent and developing it with water. 90
8. The process of preparing pictures to be produced by tanning action consisting in applying a mixture of a diazo compound containing besides the diazo group a basic group, an organic colloid and a pigment on a base placing the object to be copied on the layer sensitive to light, exposing it to light, treating it with a tanning agent and developing it with water. 95
9. The process of preparing pictures to be produced by tanning action consisting in applying a mixture of a diazo compound containing besides the diazo group a basic group, an organic colloid, a pigment and a stabilizer on a base, placing the object to be copied on the layer sensitive to light, exposing it to light, treating it with a tanning agent and developing it with water. 100
10. The process of preparing pictures to be produced by tanning action consisting in applying a mixture of a diazo compound containing besides the diazo group a basic group and an organic colloid on a base placing the object to be copied on the layer sensitive to light, exposing it to light, treating it with a solution of a chromate and developing it with water. 105
11. The process of preparing pictures to be produced by tanning action consisting in applying a mixture of a diazo compound containing besides the diazo group a basic group, an organic colloid and a pigment on a base placing the object to be copied on the layer sensitive to light, exposing it to light, treating it with a solution of a chromate and developing it with water. 110
12. The process of preparing pictures to be produced by tanning action consisting in applying a mixture of a diazo compound containing besides the diazo group a basic group, an organic colloid, a pigment and a stabilizer on a base placing the object to be copied on the layer sensitive to light, exposing it to light, treating it with a solution of a chromate and developing it with water. 115
13. The process of preparing pictures to be produced by tanning action consisting in applying a mixture of the diazo compound of the 1,4-amino-monoethyl-naphthylamine, an organic colloid, a pigment and a stabilizer on a base placing the object to be copied on the layer sensitive to light, exposing it to light, treating it with a solution of a chromate and developing it with water. 120
14. The process of preparing pictures to be produced by tanning action consisting in applying a diazo compound on a base placing the object to be copied on the layer sensitive to light, exposing it to light, pressing it on a layer of an organic colloid, having been treated with a solution of a chromate and developing it with water. 125
15. The process of preparing pictures to be produced by tanning action consisting in applying a mixture of a diazo compound and a pigment on a base placing the object to be copied on the layer sensitive to light, exposing it to light, pressing it on a layer of an organic colloid, having been treated with a solution of a chromate and developing it with water. 130
16. The process of preparing pictures to be produced by tanning action consisting in applying a diazo compound containing besides the diazo group a basic group on a base placing the object to be copied on the layer sensitive to light, exposing it to light, pressing it on a layer of an organic colloid, having been treated with a solution of a chromate and developing it with water. 135
17. The process of preparing pictures to be produced by tanning action consisting in applying a mixture of a diazo compound containing besides the diazo group a basic group and a pigment on a base placing the object to be copied on the layer sensitive to light, exposing it to light, pressing it on a layer of an organic colloid, having been

treated with a solution of a chromate and developing it with water.

18. The process of preparing pictures to be produced by tanning action consisting in applying a mixture of the diazo compound of 1,4-amino-monoethyl-naphthylamine and a pigment on base placing the object to be copied on the layer sensitive to light, exposing it to light, pressing it on a layer of an organic colloid, having been treated with a solution of a chromate and developing it with water.

In testimony whereof, we affix our signatures.

- 15 MAXIMILIAN PAUL SCHMIDT.  
RUDOLF ZAHN.  
WILHELM KRIEGER.

#### CERTIFICATE OF CORRECTION.

Patent No. 1,762,033.

Granted June 3, 1930, to

MAXIMILIAN PAUL SCHMIDT ET AL.

It is hereby certified that the name of assignee in the above numbered patent was erroneously written and printed as "Halle & Co. Aktiengesellschaft, whereas said name should have been written and printed as Kalle & Co. Aktiengesellschaft, as shown by the records of assignments in this office; and that the said Letters Patents should be read with this correction therein that the same may conform to the record of the case in the Patent Office.

Signed and sealed this 2nd day of September, A. D. 1930.

M. J. Moore,  
Acting Commissioner of Patents.

(Seal)

45

50

55

60

65

treated with a solution of a chromate and developing it with water.

18. The process of preparing pictures to be produced by tanning action consisting in applying a mixture of the diazo compound of 1,4-amino-monoethyl-naphthylamine and a pigment on base placing the object to be copied on the layer sensitive to light, exposing it to light, pressing it on a layer of an organic colloid, having been treated with a solution of a chromate and developing it with water.

In testimony whereof, we affix our signatures.

- 15 MAXIMILIAN PAUL SCHMIDT.  
RUDOLF ZAHN.  
WILHELM KRIEGER.

#### CERTIFICATE OF CORRECTION.

Patent No. 1,762,033.

Granted June 3, 1930, to

MAXIMILIAN PAUL SCHMIDT ET AL.

It is hereby certified that the name of assignee in the above numbered patent was erroneously written and printed as "Halle & Co. Aktiengesellschaft, whereas said name should have been written and printed as Kalle & Co. Aktiengesellschaft, as shown by the records of assignments in this office; and that the said Letters Patents should be read with this correction therein that the same may conform to the record of the case in the Patent Office.

Signed and sealed this 2nd day of September, A. D. 1930.

M. J. Moore,  
Acting Commissioner of Patents.

(Seal)

45

50

55

60

65